

Feb. 4, 1964

M. F. McDONALD, SR., ETAL 3,120,494

CATALYST COMPOSITION AND PROCESS FOR IMPREGNATING

A SUPPORT FOR AN  $AlBr_3$ -CATALYZED REACTION

Filed Sept. 3, 1959

3 Sheets-Sheet 1



FIGURE 1

Michael Francis McDonald, Sr. INVENTORS  
Earl Joseph Estopinal, Jr.

BY *Richard H. Nagel*

PATENT ATTORNEY

Feb. 4, 1964

M. F. McDONALD, SR., ETAL 3,120,494

CATALYST COMPOSITION AND PROCESS FOR IMPREGNATING

A SUPPORT FOR AN  $AlBr_3$ -CATALYZED REACTION

Filed Sept. 3, 1959

3 Sheets-Sheet 2

FIGURE 2  
EFFECT OF HBr ON  $AlBr_3$  ADSORPTION  
PILOT UNIT (CONTINUOUS) & BATCH DATA

CONDITIONS - 2-20 WT. %  $AlBr_3$ , ALUMINA SUPPORT  
100° F.



Michael Francis McDonald, Sr. INVENTORS  
Earl Joseph Estopinal, Jr.

BY *Richard J. Nagel*

PATENT ATTORNEY

Feb. 4, 1964

M. F. McDONALD, SR., ETAL 3,120,494  
CATALYST COMPOSITION AND PROCESS FOR IMPREGNATING

A SUPPORT FOR AN  $AlBr_3$ -CATALYZED REACTION

Filed Sept. 3, 1959

3 Sheets-Sheet 3

FIGURE 3

EFFECT OF  $AlBr_3$  CONCENTRATION & V/V/HR. ON ADSORPTION RATE  
CONTINUOUS PILOT UNIT DATA

CONDITIONS- 100°F, ALUMINA SUPPORT, CONSTANT HBr



Michael Francis McDonald, Sr. INVENTORS  
Earl Joseph Estopinal, Jr.

BY *Richard W. Nagel*

PATENT ATTORNEY

3,120,494

CATALYST COMPOSITION AND PROCESS FOR IMPREGNATING A SUPPORT FOR AN  $AlBr_3$ -CATALYZED REACTION

Michael Francis McDonald, Sr. and Earl Joseph Estopinal, Jr., Baton Rouge, La., assignors to Esso Research and Engineering Company, a corporation of Delaware

Filed Sept. 3, 1959, Ser. No. 837,845  
8 Claims. (Cl. 252—442)

This invention concerns improvements in the catalytic treatment of paraffin hydrocarbons. More particularly, the invention relates to improvements in the liquid phase conversion of normal or slightly branched chain hydrocarbons to commercially valuable, more highly branched isomers, employing aluminum bromide as the catalyst. Still more particularly, the present invention relates to improvements in the starting up of a reactor for carrying out the process on a commercial scale.

It is well known that the more highly branched isomers of the paraffinic hydrocarbons occurring in petroleum gasoline fractions are more valuable than the corresponding slightly branched or straight chain hydrocarbons because of their higher octane ratings. The demand for motor fuels of greater octane number has increased markedly as the automotive industry has provided gasoline engines with increasingly higher compression ratios to attain greater efficiency. One of the economically important ways in which the increased demands for high octane fuels can be met is through the isomerization of the light naphtha components of such fuels.

It may be generally stated that the isoparaffinic and branched chain paraffin hydrocarbons are of greater commercial value to the petroleum industry than the corresponding straight chain hydrocarbons. Thus, for example, 2,2-dimethylbutane has a higher octane rating than the isomeric normal hexane. Isobutane is more valuable than normal butane since the former can be used as the basis for the preparation of 8-carbon-atom branched chain hydrocarbons by alkylation with butylene.

The isomerization of normal paraffin hydrocarbons of from 4 to 7 carbon atoms into the corresponding branched chain homologs is well known. For effecting the isomerization, it is customary to employ certain metal halides, particularly aluminum chloride or aluminum bromide, in conjunction with certain promoters, such as hydrogen chloride, hydrogen bromide or boron fluoride. Insofar as the isomerization of light naphthas is concerned, the lower the temperature of isomerization, within limits, the more favorable is the equilibrium for converting straight chain paraffin hydrocarbons into isomers of high octane rating. Aluminum bromide has been found to be more active than aluminum chloride at lower isomerization temperatures, e.g., in the range of about 50° to about 120° F.

Aluminum bromide is also known to be an active catalyst for the alkylation of isoparaffinic hydrocarbons with olefinic hydrocarbons to produce branched chain hydrocarbons that are useful motor fuel components. The same catalyst, with suitable promoters, can be employed to effect the liquid phase reaction of paraffin hydrocarbons of from 6 to 18 carbon atoms with isobutane or isopentane at temperatures of about 30° F. to about 120° F. to give products predominating in  $C_5$  to  $C_7$  branched chain hydrocarbons of high octane rating; in a process involving simultaneous cracking, isomerization and alkylation reactions.

One disadvantage in the use of aluminum bromide in reactions of the types outlined above is that it is appreciably soluble not only in the products of those reactions, but also in the starting materials. Because of this, prac-

tical means must be available not only for recovering the aluminum bromide from the reaction products so that it can be reused in the reaction, but also means must be taken to maintain catalyst in the active state in the reactor at all times. This is particularly difficult, for reasons set forth below, during the start-up of the operation.

A peculiarity of the aluminum bromide catalyzed hydrocarbon isomerization reaction is the fact that an activator, usually an oxygen containing material must be present to

cause the reaction to proceed. Without them, the reaction will not go. These activators may be solid supports, such as bauxite, alumina, molybdena, silica gel, or similar materials; likewise, many liquid oxygen containing compositions, such as alcohols, ethers, organic and inorganic acids, carboxyl compounds and the like, have been found to a greater or less extent to function as activators. These activators probably form molecular complexes with the  $AlBr_3$  or its dimer,  $Al_2Br_6$  and it is the complex that actually functions as the catalytic agent.

20 A still further peculiarity about the  $AlBr_3$  catalyzed liquid phase hydrocarbon reaction systems is the fact that the catalyst must be present in two phases or species, namely  $AlBr_3$  associated with the activator or support, this forming a solid phase when a solid support is em-

25 ployed, and  $AlBr_3$  or  $Al_2Br_6$  dissolved in the reactant hydrocarbon. Again, it has been found that supported  $AlBr_3$  will not catalyze the liquid phase isomerization or isoparaffin alkylation process in the absence of dissolved  $AlBr_3$ . Furthermore, after a support has become sat-

30 urated, as with 80 to 100% of its weight of  $AlBr_3$ , it will not isomerize hydrocarbons if free  $AlBr_3$  is cut out of the feed. Normally, a catalyst support, such as Porocel, which is a calcined bauxite, adsorbs about 30 to 70% by weight of  $AlBr_3$  from the solution. This means when 35 starting up a commercial isomerization reactor, the reactor support, such as Porocel, alumina, molybdena and the like, must have 30 to 70% by weight of  $AlBr_3$  adsorbed before catalyst activity is stabilized.

The efficiency and technique of adsorbing this  $AlBr_3$  40 on a commercial reactor bed is extremely important from an economic standpoint. Thus, a 20,000 bd./d. isomerization unit with a design feed rate of 0.1 to 0.2 v./v./hr. will require from \$300,000 to \$800,000 worth of  $AlBr_3$  deposited on the reactor bed. Even when catalyst re- 45 cycle is employed, the maximum feed rate is about 0.6 to 0.8 v./v./hr., and  $AlBr_3$  cost would then be between \$50,000 and \$200,000.

It is an important object of the present invention to 50 present a process for starting up a liquid phase  $AlBr_3$  isomerization and isoparaffin alkylation unit with high degree of efficiency enabling normal isomerization reaction to proceed under substantially equilibrium conditions in a minimum period of time and with a maximum degree of effectiveness.

55 Other and further objects and advantages of the present invention will be more clear hereinafter.

In accordance with the present invention it has been found that the highest rates of  $AlBr_3$  adsorption (w. 60  $AlBr_3$ /hr./w. support) are obtained during start-up by having a feed composition of 2 to 20 wt. percent  $AlBr_3$ , and 5 to 20 wt. percent HBr (based on total feed) and operating at 0.5 to 10 v./v./hr. Recycling the hydrocarbon feed stream, composed of isobutane and/or naphthalenes, both of which components are reactants in the isomerization process, and the dissolved  $AlBr_3$  and HBr across the reactor beds at the described v./v./hr. is critical to insure maximum utilization of feed additives. Both the isobutane and the naphthalenes, i.e., methylcyclopentane, cyclohexane and methylcyclohexane, are cracking inhibitors and prevent catalyst degradation and fouling.

70 Furthermore, to provide maximum efficiencies, recycle

conditions include liquid feed rates (AlBr<sub>3</sub> dissolved in naphthenes and/or i-C<sub>4</sub>) of 0.5 to 10 v./v./hr., an AlBr<sub>3</sub> concentration of 2 to 20 wt. percent based on feed, and a 5 to 20 wt. percent HBr concentration, based on feed. HBr serves not only to promote the isomerization reaction but also to stabilize the AlBr<sub>3</sub> and aids in keeping it in solution. At the start-up, of course, the reactor is packed with the fresh activator, such as Porocel, alumina and the like.

The process of the present invention may be illustrated diagrammatically in FIGURE 1 of the accompanying drawings, wherein 2 represents an isomerization reactor during the start-up stage. This reactor may be packed with the activators previously mentioned. In order to deposit the desired quantity of AlBr<sub>3</sub> on this activator bed, a stream of AlBr<sub>3</sub> dissolved in naphthenes or isobutane, or in a mixture of both, is admitted through lines 24 and 12 into reactor 2. As indicated previously, the AlBr<sub>3</sub> concentration is 2 to 20% by weight; and the solution is circulated through the reactor and the pump-around system by means of pump 6 until the reactor support carries 30 to 70 wt. percent AlBr<sub>3</sub>. Further admitted through lines 24 and 12 is 5 to 20% by weight of HBr, based on feed. Preferably the temperature within reactor 2 is about 60° to 150° F., and a pressure of 10 to 150 p.s.i.g. is maintained. The feed rate must be maintained at least at 0.5 v./v./hr. for high efficiency.

As shown in FIGURE 3 the relative adsorption rates are for the most part constant after 0.5 v./v./hr. Operating at rates less than 0.5 v./v./hr. would greatly increase the time necessary to saturate the support by limiting the amount of AlBr<sub>3</sub> in contact with the support. There is no advantage for operation above 3 v./v./hr.

An excellent method of providing AlBr<sub>3</sub> in a highly active form for this process is to synthesize it in situ. For this purpose, a portion of the stream from pump 6, comprising isobutane and/or naphthenes as well as HBr, is passed over a bed of aluminum ribbon or turnings or the like and AlBr<sub>3</sub> in high purity is withdrawn in solution from zone 16 through line 18.

When sufficient AlBr<sub>3</sub> is built up within the reactor 2, valve 22 is closed, valve 20 opened, and the system is now in readiness for the isomerization reaction proper. The latter, not being a part of the present invention, is not here illustrated, but it includes passage of a C<sub>5</sub>-C<sub>7</sub> normal hydrocarbon stream to reactor 2 and passage of isomerization product through line 34 to a conventional recovery system.

The critical nature of the variables that must be maintained to obtain saturation of the support in a short time is clearly shown in the curves in FIGURES 2 and 3.

FIGURE 2 shows that saturation of the support is achieved in a far shorter period of time at the higher HBr concentration levels than at the lower. FIGURE 3 indicates the upper limit of AlBr<sub>3</sub> concentration and space velocity, above which no advantages are realized.

That it would be economically undesirable to employ a once-through operation for saturating the support is shown in Table I. The last column shows the amount

of AlBr<sub>3</sub> which passes out of the reactor with the effluent. Thus if the total AlBr<sub>3</sub> adsorbed in a commercial unit costs about \$500,000, then operation 1 would lose \$43,000 during the start-up; 2 would lose \$780,000; and operation 3 would lose \$294,000. This is calculated from the equation:

$$\$ \text{ lost} = \left[ \frac{500,000}{100 - \text{percent AlBr}_3 \text{ lost}} - \$500,000 \right]$$

Table I  
ONCE-THROUGH AlBr<sub>3</sub> ADSORPTION

| Operation | CONDITIONS |                                         |                          |            | AlBr <sub>3</sub> Lost, Percent on Total AlBr <sub>3</sub> Fed to Reactor |
|-----------|------------|-----------------------------------------|--------------------------|------------|---------------------------------------------------------------------------|
|           | V./V./Hr.  | AlBr <sub>3</sub> , Wt. Percent in Feed | HBr, Wt. Percent in Feed | Temp., °F. |                                                                           |
| 1         | 1.2        | 0.8                                     | 9                        | 100        | 8                                                                         |
| 2         | 3.2        | 4.1                                     | 9                        | 100        | 61                                                                        |
| 3         | 0.5        | 6.6                                     | 0                        | 100        | 37                                                                        |

What is claimed is:

1. A process for impregnating a support for an AlBr<sub>3</sub>-catalyzed reaction which comprises passing to an oxide support a hydrocarbon solution containing from 2 to 20% by weight of AlBr<sub>3</sub> at a rate of 0.5 to 10 v./v./hr., further passing to said support 5 to 20 weight percent of HBr, based on hydrocarbon, and recycling said product until said support is saturated with aluminum bromide.
2. The process of claim 1 wherein said support is calcined bauxite.
3. The process of claim 1 wherein said support is alumina.
4. The process of claim 1 wherein said hydrocarbon is isobutane.
5. The process of claim 1 wherein said hydrocarbon comprises naphthenic hydrocarbon compounds.
6. The process of claim 1 wherein adsorption conditions include temperatures of 60° to 150° F. and pressures of from 10 to 150 p.s.i.g.
7. An improved process for saturating an oxide support with AlBr<sub>3</sub> which comprises recycling to said bed a 2 to 4% by weight solution of AlBr<sub>3</sub> in a hydrocarbon selected from the class consisting of isobutane and naphthenes, further maintaining on said bed an HBr concentration of about 8 to 10% by weight of hydrocarbon, and maintaining a recycle rate of about 0.5 to 3 v./v./hr.
8. The process of claim 1 wherein at least a portion of said recycle stream is passed through a bed of aluminum to synthesize further amounts of AlBr<sub>3</sub>.

References Cited in the file of this patent

UNITED STATES PATENTS

- |           |                |       |               |
|-----------|----------------|-------|---------------|
| 2,265,548 | Schuit         | ----- | Dec. 9, 1941  |
| 2,410,894 | Montgomery     | ----- | Nov. 12, 1946 |
| 2,446,100 | Oblad et al.   | ----- | July 27, 1948 |
| 2,971,037 | Gilbert et al. | ----- | Feb. 7, 1961  |